

# UNITED STATES PATENT OFFICE.

LORENZO L. CROUNSE, OF KINGSTON, NEW YORK.

## IMPROVEMENT IN THE UTILIZATION OF THE DUST OR CULM OF ANTHRACITE COAL AS FUEL.

Specification forming part of Letters Patent No. **222,466**, dated December 9, 1879; application filed November 15, 1879.

*To all whom it may concern:*

Be it known that I, LORENZO L. CROUNSE, of Kingston, in the county of Ulster and State of New York, have invented certain new and useful Improvements in the Utilization of the Dust or Culm of Anthracite Coal as a Fuel; and I do hereby declare the following to be a full, clear, and exact description of the invention, such as will enable others skilled in the art to which it appertains to make and use the same.

Whereas the undersigned did by deed of assignment before issue, on record in the Patent Office, secure on the 20th of April, 1875, and 5th of December, 1876, Letters Patent—viz., 162,362, 162,363, and 185,090—for an improvement in process and machinery for the manufacture of artificial fuel, under which patents he has since been continually engaged in said manufacture; and whereas the practical manipulation of anthracite-coal dust or culm has demonstrated that, owing to its inherent vitreous character, it is difficult to so combine it with any fusing material so far tried as to prevent attrition to the machinery in the manufacture or decrepitation in combustion, thus failing to secure the great calorific power absolutely contained in its excessive carbon—

Now be it known that I have devised an improvement in said process which overcomes said difficulty, and which improvement relates especially to the more successful utilization of the culm or dust of anthracite coal as a fuel, and I respectfully ask the issue of Letters Patent of the United States covering the same.

The improvement which I claim as my invention is described as follows:

To the proportions of the volume of coal-tar pitch and anthracite-coal dust, as heretofore used, which are usually about ten per cent. of pitch to ninety per cent. of dust, I add from fifteen to thirty per cent.—though I do not limit myself to these exact proportions—of the slack or dust of bituminous or semi-bituminous coal, which combination is effected in the following manner.

The bituminous slack or dust, being placed in a separate receptacle, is fed in the requisite proportions, by a screw or worm feed with blades or arms of the proper mechanical pitch and

diameter, or in any other suitable manner, into the same hopper or chute with the pitch, where the two materials are first thoroughly mixed, and from which they move rapidly into a half-open cylinder or semicircular mixer, or any other suitable vessel for mixing, where they meet the volume of anthracite dust or culm, and all the materials are thus thoroughly mixed in the dry state. They next pass into a longitudinal steam-jacketed cylinder, where they are subjected to fusion by steam superheated to a temperature of from 500° to 700°. This high heat not only melts the pitch, but volatilizes the lighter elements in the bituminous or semi-bituminous slack, which assists the binding effect of the pitch. The materials are then taken by an elevator from the mouth of this cylinder, carried up and dumped into another and preferably upright cylinder, where a further fusion and mixture take place, where more steam of the same or lesser temperature is added, if necessary, and from which the mass of materials thus prepared passes to the compression or molding table, where they are compressed into cubes, spheres, or parallelograms. The addition of the bituminous or semi-bituminous dust or slack gives, by its softer nature and its tarry, oily, and paraffine elements, increased firmness and tenacity to the product, and also increases the coking effect in combustion, so that the anthracite dust or culm is thoroughly consumed, and its high calorific power completely utilized.

What I claim as my invention is—

The combination, by process as above described, of the coal-tar pitch, slack, or dust of bituminous or semi-bituminous coal with the dust or culm of anthracite coal, under the conditions of dry mixture, subsequent high heat, mixture, and compression producing a coking or semi-coking fuel, substantially as described and set forth; and I also claim the fuel as thus produced.

In testimony that I claim the foregoing I have hereunto set my hand this 15th day of November, 1879.

LORENZO L. CROUNSE.

Witnesses:

L. DEANE,  
C. S. DUBOIS.